

# United States Patent [19]

Sawtell et al.

[11] Patent Number: 4,689,090

[45] Date of Patent: Aug. 25, 1987

[54] SUPERPLASTIC ALUMINUM ALLOYS  
CONTAINING SCANDIUM

[75] Inventors: Ralph R. Sawtell, Emeryville, Calif.;  
Philip E. Bretz; Craig L. Jensen, both  
of Plum Boro, Pa.

[73] Assignee: Aluminum Company of America,  
Pittsburgh, Pa.

[21] Appl. No.: 841,648

[22] Filed: Mar. 20, 1986

[51] Int. Cl.<sup>4</sup> ..... C22F 1/04

[52] U.S. Cl. ..... 148/2; 148/11.5 A;  
148/415; 148/437; 420/902

[58] Field of Search ..... 148/2, 11.5 A, 12.7 A,  
148/415-418, 437-440; 420/902

## [56] References Cited

### U.S. PATENT DOCUMENTS

3,619,181 11/1971 Willey ..... 148/415

Primary Examiner—R. Dean  
Attorney, Agent, or Firm—Carl R. Lippert

## [57] ABSTRACT

Superplastic forming of aluminum work stock is improved by including therein about 0.05% to about 10% or 15% scandium. In preferred practices, soluble elements such as magnesium are also included in the aluminum alloy.

15 Claims, 2 Drawing Figures





FIG.1



FIG.2

**SUPERPLASTIC ALUMINUM ALLOYS  
CONTAINING SCANDIUM**

**FIELD OF INVENTION**

This invention relates to superplastic forming of aluminum alloys and to special aluminum alloys and products adapted to superplastic forming at elevated temperature.

**BACKGROUND OF THE INVENTION**

Superplastic forming of metals is well known in the art whereby complex shapes are formed from metal at elevated temperature utilizing the superplastic forming characteristics of the metal to avoid tearing and other problems in forming complex shapes. Superplastic forming can be viewed as an accelerated form of high-temperature creep and occurs much like sagging or creep forming. In the case of aluminum alloys, superplastic forming is normally performed at temperatures above 700° F., typically in the range of about 900° to 1000° F. or a little higher. At this temperature, the metal creeps and can be moved by shaping operations at relatively low stress levels, the stress at which the metal starts to move easily or flow being referred to as the "flow stress". Superplastic forming is recognized as being able to produce intricate forms or shapes from sheet metal and offers the promise of cost savings. For instance, an airplane member previously made by stamping several parts from sheet and then joining the separate parts together into a more complex shape can be formed from a single piece of metal by superplastic forming techniques. However, the superplastic forming techniques themselves are time-consuming in that like any form of creep forming, the metal flowing operation proceeds relatively slowly in comparison with high-speed press forming. Substantial cost-savings and benefits could be realized if the aluminum alloy to be superplastically formed could be made to flow faster at a given temperature or be superplastically formed at a lower temperature or both without tearing or rupturing.

There are a number of approaches taken to enhance superplastic forming. Some of these approaches are directed to manipulations in the superplastic forming operation to enhance that operation or alleviate problems therein largely by controlling the flow of the metal during forming. Examples of such are shown in U.S. Pat. Nos. 3,997,369, 4,045,986, 4,181,000, and 4,516,419, all incorporated herein by reference. Another approach is directed to the metal to be superplastically formed. It has long been recognized that fine grain size enhances forming operations including superplastic forming operations. Some examples of efforts to achieve fine grain size are shown in U.S. Pat. Nos. 3,847,681 and 4,092,181. One approach to achieving fine grain size which was old as far back as the 1960's includes imparting substantial working effects such as cold work to aluminous metal followed by rapid heating to recrystallization temperature. However, despite the various approaches taken to improve either the superplastic forming operation or the metal stock going into the operation, there remains substantial room for improvement and an alloy which would enable the superplastic forming operation to proceed faster or at a lower temperature is both desirable and sought after.

**SUMMARY OF THE INVENTION**

In accordance with the invention, the superplastic forming performance of aluminum alloys is greatly enhanced by the addition thereto of small but effective amounts of the element scandium, for instance amounts in the range of 0.05 to 10%, preferably 0.1 to 5%. When additions above the maximum solid solubility are used (about 0.4 weight percent for the Al-Sc binary alloy), it will be appreciated that some form of rapid solidification should be used in casting or solidifying the alloy to avoid the formation of large and ineffective intermetallic constituents. The scandium addition is especially beneficial when the aluminum alloy contains a soluble element such as magnesium as explained hereinbelow. In accordance with the invention it has been found that elongation levels substantially exceeding 1000% can be achieved at temperatures as low as 750° F. and strain rates of 0.01 sec<sup>-1</sup> (1.0% per second). This performance translates into taking minutes to do what previously took hours and has to be considered remarkable by any standard, and is considered to greatly enhance superplastic forming of aluminous alloys. Such performance has been sought after in the aluminum superplastic forming art and is the subject of considerable government and privately funded research. Equally significant is the fact that the addition of scandium does not otherwise harm the performance of the aluminum alloy at the lower service temperatures normally used for aluminum alloys in structural applications. For instance, as indicated in U.S. Pat. No. 3,619,181, incorporated herein by reference, scandium can be included in aluminum alloys to improve strength properties at room and temperatures of about 149° C. (about 300° F.) and even up to temperatures up to 260° C. (about 500° F.). Accordingly, it was most surprising to see that this effect would practically reverse at superplastic forming temperatures wherein the addition of scandium weakens the metal in the sense of reducing the flow stress, that is, the stress applied to the metal to make it flow in superplastic forming operations.

**THE DRAWINGS**

Reference herein is made to the drawings, in which: FIG. 1 is a graph plotting true strain rate versus longitudinal elongation.

FIG. 2 is a graph plotting strain rate sensitivity parameter "M" versus true strain rate.

**DETAILED DESCRIPTION**

The amount of scandium included in aluminum alloys in the practice of the invention ranges from a minimum of about 0.05% up to a maximum as high as 10% or even possibly higher, for instance up to 15%, if rapid solidification casting techniques are used, although it is preferred to employ a maximum of about 5% scandium or less for economic reasons. All composition percentages herein are by weight, and it is to be understood that aluminum alloys refer to aluminum metal containing greater than 50% aluminum, for instance, at least 60% aluminum. A suitable range for scandium is about 0.1 or 0.2 up to about 0.9 or 1% scandium. Within this range, the benefits of scandium are achieved at what is considered very reasonable cost, especially when the extent of the advantages is appreciated. One preferred scandium range is about 0.3 to about 0.7%.

In addition to scandium, it is preferred that the aluminum alloy contain one or more elements which are in

solid solution at superplastic forming temperature and which, in combination with Sc, lower its flow stress at superplastic forming temperature. Accordingly, the aluminum alloy contains selected amounts of one or more of the elements magnesium, silicon, copper, silver, germanium, lithium, manganese, or zinc in an amount, typically 0.1% or more, that provides at least some of the element in solid solution at superplastic forming temperature and which alters the flow stress of the scandium-containing aluminous metal at superplastic forming temperature. The amounts for these elements, broadly stated, are up to 10% Mg, up to 2% Si, up to 10% Ag, up to 5% Cu, up to 5% Ge, up to 5% Li, up to 1.5% Mn, and up to 10% Zn. Of this group, a presently preferred embodiment includes magnesium present in amounts of 1 to 7 or 8%, with amounts of 2 to 6% being considered to render good performance and amounts of 3 to 5% Mg, preferably 3.5 to 4.5% Mg, offering quite impressive performance in accordance with the invention.

In addition to the elements recited above, the aluminous metal can also contain other elements such as Fe, Co, Ni, Zr, rare earth elements, or various other elements associated with aluminum and aluminum alloys as conscious additions or as incidental elements or as impurities, although, as indicated above, a presently preferred embodiment is an aluminum alloy containing about 3 to 5% Mg and about 0.2 to 0.8% Sc along with incidental elements and impurities. Constituents (intermetallic compounds) or phases which are insoluble at superplastic forming temperature can interfere or cause defects in superplastic forming. Accordingly, elements are preferably avoided in amounts or in combinations which favor formation of constituents at superplastic forming temperature. The amount of such an element tolerated depends in part on the rate of solidification and of heating employed in operations prior to superplastic forming. For instance, extremely rapid solidification of cast stock about 0.150-inch thick followed by cold rolling and rapid heating to superplastic forming temperature and fairly rapid superplastic forming can avoid formation of the relatively large insoluble phases which interfere with superplastic forming.

Silicon is an example of an element which can form insoluble phases and one preferred embodiment favors limiting Si to a maximum of 0.4 or 0.45% or possibly 0.5%, preferably 0.25% maximum especially where magnesium is present in the alloy. Other examples of elements which can form intermetallic compounds and phases which interfere with superplastic forming are Ca, Ti, V, Cr, Fe, Co, Ni, cerium, and the rare earth elements and the refractory elements such as Ta, W, Re, Mo, and Nb.

Soluble elements such as Zn, Cu, and Mg also can form insoluble constituents where one or more is present. For example, Cu and Mg can form constituents if both are present in sufficient amounts and processing temperatures favor precipitation.

One of the aspects observed in practicing some embodiments of the invention is the relation between the scandium-aluminum phase, believed to be approximately  $Al_3Sc$ , and the aluminum matrix in that the scandium-aluminum phase appears to be coherent with the aluminum phase, that is, having a crystal structure very similar to the aluminum phase such that the scandium-aluminum phase can be less pronounced or contrasted with the aluminum matrix than other phases appearing in various aluminum alloys. Because the aluminum-

scandium phase has a structure very similar to that of the aluminum matrix, it is relatively stable at elevated temperatures and tends to resist coarsening during superplastic forming. The presence of this phase appears to prevent classical recrystallization from occurring during superplastic forming. The term "classical recrystallization" as used herein refers to the phenomenon wherein crystal growth occurs about nucleation sites and wherein the original crystal or grain boundaries as well as sub-grain structures within those boundaries substantially disappear and are replaced by substantially whole crystal grains with new grain boundaries.

The improved superplastic forming metal can be produced in accordance with methods used in producing other aluminum alloys in that, depending on the Sc content chosen, the alloy is readily castable into ingot, including thin ingot, such as by semi-continuous or continuous casting techniques, the latter including the various belt or drum casting techniques. In general, higher Sc content suggests smaller ingot size or higher chill rates in casting, or both. In a presently preferred embodiment of the invention, where Sc contents of about 0.2 to 0.8 are used, some form of mildly rapid solidification is desirable to obtain the best possible distribution of Sc-bearing phases. Chill rates of 15° C. or 20° C. (36° F.) per second or faster are generally preferred. One way to achieve this condition is to cast relatively thin ingot such as not over 4 inches thick, for instance about 1 or 2 inches thick. Higher Sc content preferably is accommodated with faster casting chill rates. The solidification rate desired is related to the presence of certain other elements in addition to Sc. As a general rule, the greater the content of elements other than aluminum, especially elements which form intermetallic phases insoluble at superplastic forming temperature, the higher the desired casting chill rate.

It is desirable to impart work into the metal to break up the cast structure and alter the grain texture. Accordingly, ingot is hot rolled then cold rolled, although a thin-cast alloy such as an alloy cast to a thickness of  $\frac{1}{8}$  inch or the like can dispense with hot rolling and go directly to cold rolling. In producing aluminous metal in accordance with the invention, it is preferred that the alloy be rolled to a reduction of at least 30%, typically 90% or more. This breaks up the cast structure and strengthens the alloy. The working can be relatively hot (550° F. to 750° F.) or cold or both. Working can include rolling or extrusion, forging or other working operations. While working is preferred, it may be possible in some cases that the as-cast stock can be superplastically formed.

The  $Al$ - $Mg$ - $Sc$  alloy does not require a high temperature preheat before working when cast in thin ingot. Heating to 550° F. before hot working is adequate. One preferred practice includes hot working at the lowest temperature usable without excessive break-up of the working stock. The preferred  $Al$ - $Mg$ - $Sc$  alloys are considered heat-treatable alloys and some precipitation of the  $Al_3Sc$  can occur during hot rolling. Higher amounts of Sc or higher amounts or numbers of precipitate-forming elements further favor the use of lower working temperatures and shorter times at elevated temperature.

It is desired to perform any hot rolling above 550° F. to avoid cracks, but it is preferred to keep hot rolling temperatures not exceeding 800° F. or preferably not above 750° F. to help avoid modifying or coarsening the  $Al_3Sc$  phase to the extent of possibly degrading super-

plastic forming performance. That is, while the Al-Sc phase is relatively stable at elevated temperatures, it is considered preferable to avoid substantial periods of time at temperatures above 800° F. in producing the alloy product.

It is believed that the addition of Sc will improve the superplastic forming performance of alloys such as 7475, which are now considered to have superplastic characteristics. However, alloys such as 7475 whose Aluminum Association sales limits are 5.2 to 6.2% Zn, 1.9 to 2.6% Mg, 1.2 to 1.9% Cu, 0.18 to 0.25% Cr, balance Al and incidental elements and impurities, and others which include precipitate-forming elements are preferably processed by operations which do not favor formation of precipitates which are insoluble at superplastic forming temperature. The 7475 alloy would be brought to superplastic forming temperature, about 940° F. to 960° F., and formed into the desired shape. Since a 950° F. forming temperature is suited for solution heat treating this alloy, it can be quenched and aged right after forming.

From the preceding, it can be seen that preferred operations in processing the selected alloy composition into a wrought product include casting at high or fairly high chill rates to produce work stock. Working, including associated heating, is preferably carried out at lower temperatures or at moderate elevated temperatures, for instance 550° F. to 750° F. or 800° F., to reduce formation of undesired precipitated phases. Higher temperatures are less preferred but usable if employed for short enough time to avoid undesired precipitates. The preferred practices are more important where elements are present in the alloy which tend to produce precipitates which are insoluble or agglomerate at superplastic forming temperature sufficiently to interfere with the subsequent superplastic forming operation.

#### EXAMPLE I

In order to demonstrate the improvement achieved according to the practice of the invention, the following illustrative Example proceeds. Alloys of various compositions indicated in Table I were semi-continuously cast at relatively high chill rates into ingots 1inch × 6-inches and 2½ inches × 12-inch in cross-section and then hot and cold rolled into sheet about 0.1-inch thick. The hot rolling operation at 550° F. produced a sheet of about 0.25-inch thick which was cold rolled to a final gauge of 0.1 inch, a cold reduction of 60%. Without a separate annealing or recrystallization treatment, the sheet was heated to temperatures of 750° F. in some cases and 1000° F. in other cases for superplastic property measurement. The flow stress and elongation were measured at both temperatures and are listed in Table I.

TABLE I

| Alloy        | Strain Rate       |              | Temperature<br>°F. | Flow Stress |     | Elongation<br>% |
|--------------|-------------------|--------------|--------------------|-------------|-----|-----------------|
|              | sec <sup>-1</sup> | % per second |                    | KSI         | MPA |                 |
| Al-0.5Sc     | .01               | 1%           | 750                | 7.8         | 54  | 92              |
| Al-0.5Sc     | .002              | 0.2%         | 1000               | 1.5         | 10  | 157             |
| Al-4Mg       | .01               | 1%           | 750                | 6.7         | 46  | 194             |
| Al-4Mg       | .002              | 0.2%         | 1000               | 1.3         | 9   | 210             |
| Al-4Mg-0.5Sc | .01               | 1%           | 750                | 4.6         | 32  | >1050           |
| Al-4Mg-0.5Sc | .002              | 0.2%         | 1000               | 0.9         | 6   | >1050           |
| Al-6Mg-0.5Sc | .01               | 1%           | 750                | 4.9         | 34  | 341             |
| Al-6Mg-0.5Sc | .002              | 0.2%         | 1000               | 0.9         | 6   | >1050           |

From Table I it is readily clear that the alloy containing 4% magnesium and 0.5% scandium performed ex-

traordinarily well in that an elongation exceeding 1000% was achieved at both 1000° F. and 750° F. and that the flow stress level at 1000° F. was a mere 900 psi with the performance at 4% Mg in the particular test exceeding the performance level at 6% Mg. It is to be appreciated that elements such as Mg, which are soluble at superplastic forming temperatures, can be used to substantial advantage in practicing the invention. At 750° F. the superplastic forming performance of the sample containing Sc and 4% Mg substantially exceeded that of the alloy containing Sc and 6% Mg which exhibited an elongation of only 341% which, while impressive, can be considered as marginal in some situations. At 1000° F., however, the 6% Mg alloy performed quite well. Accordingly, the performance of the aluminum alloy stock can be heightened with respect to the superplastic forming temperature to optimize results both with respect to superplastic forming conditions and with respect to anticipated service requirements. 20 That is, in viewing Table I it will be apparent to those skilled in the art that while the 4% Mg alloy has superior superplastic performance at 750° F., the 6% Mg alloy at 1000° F. performs as well or better and would have greater strength at room service temperature. 25 Accordingly, the invention contemplates that additions of an element such as Mg or Cu or Zn or Li can be made in varying amounts in test specimens which (preferably after cold rolling) are tested at different superplastic forming temperatures and then the appropriate composition and superplastic forming temperature selected in accordance with the teachings of this invention to blend optimum or at least superior superplastic forming performance with service performance. In practicing the invention it has been found that the presence of an element such as Mg soluble at superplastic forming temperatures interacts somehow with Sc in improving superplastic forming performance over an aluminum-scandium alloy without the presence of such an element.

#### EXAMPLE II

The advantages of the invention can be illustrated by comparison with another superplastic forming material such as superplastic 7475 material. FIG. 1 illustrates superplastic performance plotting elongation versus true strain rate for superplastic 7475 at 960° F., a preferred superplastic forming temperature for 7475 alloy, and for the improved material containing 4% magnesium and 0.5% scandium at temperatures of 600° F., 50 750° F., 900° F., and 1000° F. The superplastic 7475 was specially processed to produce a very fine grain size and superplastic performance. The improved material was made by hot and cold rolling wherein an ingot was hot and continuously rolled to a thickness of about ¼ inch followed by cold rolling to final gauge of 0.1 inch. In

FIG. 1, the improvement performance is shown as solid lines and 7475 performance by dashed line. From FIG. 1 it is readily apparent that all of the data for the improvement are to the right side of the superplastic 7475 curve which indicates superior performance. At both 750° F. and 1000° F. the improved material facilitates a higher elongation for a given strain rate or a higher permissible strain rate for a given elongation. The data show that the improved metal has elongation at superplastic forming temperatures which is equal to or greater than that for superplastic 7475 but that higher strain rates can be used to form the improved metal. The improved superplastic metal exhibits more elongation than superplastic 7475 even when the improved alloy is strained 25 times faster than the strain rate for 7475. Further, at a strain rate of 0.01 per second (1% per second), the improved superplastic metal has many times the elongation of superplastic 7475. This highlights the superior superplasticity of the improved superplastic metal.

It has to be remembered in this connection that in superplastic forming great cost savings can be achieved if strain rate can be increased to facilitate higher production rates. Still further, at any given temperature the improvement facilitates higher strain rate and/or higher superplastic elongation. Achieving all of these benefits by adding scandium is indeed considered surprising especially when this level of performance is obtained without intricate processing steps.

It is presently believed that the basic mechanism responsible for the superplastic behavior of the improved superplastic materials may be different from the mechanism for other superplastic alloys. It is generally recognized or believed that alloys which have a strain rate sensitivity greater than 0.5 are considered good superplastic performing alloys, whereas those having a strain rate sensitivity less than 0.5 would be expected to show poor superplastic performance. However, the present improved superplastic materials can exhibit a strain rate sensitivity less than 0.5 which might, using conventional wisdom, suggest that the improved metal would not have good superplastic properties. However, the striking superior results with the improved superplastic metal would certainly defy such an impression which makes the results all the more surprising. FIG. 2 plots strain rate sensitivity parameter M versus true strain rate for the improved Al-4Mg-0.5 Sc alloy at 600° F., 750° F., 900° F., and 1000° F. (solid lines) and includes comparison with superplastic fine grain 7475 (dashed line). The strain rate sensitivity parameter M is recognized as indicating the ability of a material to distribute strain during deformation. Greater distribution of strain (higher M value) delays fracture, and it is generally considered desirable to superplastically form at a strain rate corresponding to the highest M value.

FIG. 2 illustrates further information to suggest that the mechanism responsible for the superplasticity of the improved materials may be different than for other superplastic aluminum alloys such as fine grain 7475. The maximum value of strain rate sensitivity for the improved materials occurs at a strain rate which is an order of magnitude greater than for superplastic 7475. Also, the strain rate at which the maximum strain rate sensitivity occurs does not decrease as temperature is decreased from 1000° F. to 750° F. for the improved superplastic materials, whereas experience with superplastic 7475 alloy does show such a decrease.

Another aspect of improvement shown in FIG. 2 is the relative flatness of the improvement curves as contrasted with the peaky curve for 7475. This translates to a beneficial lack of criticality for strain rate in using the improved superplastic forming materials as contrasted with 7475 whose curve peaks quickly and falls off indicating a much higher amount of sensitivity to superplastic forming rate. This lack of sensitivity to forming condition for the improved material translates to allowing forming of more complex parts, faster and with less expensive tooling.

The superplastic 7475 used for the foregoing comparison was specially processed to achieve very fine grain size which is considered to correlate with superplastic forming characteristics. Not only is the performance of the present improvement so much better than the 7475, but that performance is achieved without special fine grain processing. The grain size of the improved sheet was essentially the same as cast except that rolling had changed the grain shapes. The striking superplastic forming performance of the improved aluminum products may not fit with mechanisms considered in the art to correlate with superplastic performance. The exact mechanism responsible for the improvement is not known but may be related to some ability of Al<sub>3</sub>Sc dispersoid phases to control grain boundary motion.

While the invention has been described in terms of preferred embodiments, the claims appended hereto are intended to encompass all embodiments which fall within the spirit of the invention.

What is claimed is:

1. In a method of superplastic forming wherein aluminum alloy stock is brought to superplastic forming temperature and superplastically formed into a shaped form at superplastic forming temperature, the improvement comprising providing said aluminum alloy stock as an alloy comprising more than 50% aluminum and including 0.05 to 10% scandium.
2. In the method according to claim 1 wherein said aluminum alloy contains 0.1 to 5% scandium.
3. In the method according to claim 1 wherein said aluminum alloy contains 0.1% or more of one or more elements which are in solution at superplastic forming temperatures and which, in combination with scandium, lower the flow stress at superplastic forming temperature.
4. In the method according to claim 3 wherein said aluminum alloy contains one or more of the following elements: 0.1 to 10% Mg, 0.1 to 2% Si, 0.1 to 10% Ag, 0.1 to 5% Cu, 0.1 to 5% Ge, and 0.1 to 5% Li.
5. In the method according to claim 1 wherein said aluminum alloy contains 0.5 to 15% Mg.
6. In the method according to claim 2 wherein said aluminum alloy contains 0.1 to 1% Sc and 1 to 7% Mg and wherein at least a substantial portion of the Mg is in solid solution at superplastic forming temperature and in combination with Sc reduces the flow stress of the alloy at superplastic forming temperature.
7. In the method according to claim 3 wherein said aluminum alloy stock contains 0.1 to 5% Sc and 1 to 10% Mg and wherein at least a substantial portion of the Mg is in solid solution at superplastic forming temperature and in combination with Sc reduces the flow stress of the alloy at superplastic forming temperature and is produced by casting, hot rolling, and cold rolling said alloy to provide said stock, said hot and cold rolling operations altering the cast structure of said stock.

8. In the method according to claim 4 wherein said elements are present in amounts which do not produce precipitates which are insoluble at superplastic forming temperatures to an extent which disrupts superplastic forming.

9. In the method according to claim 8 wherein said elements are present in amounts substantially soluble at superplastic forming temperatures.

10. In the method according to claim 4 wherein the operations used to produce the superplastic forming stock are conducted to reduce the formation of said elements into phases which are insoluble at superplastic forming temperatures.

11. In the method according to claim 10 wherein said operations include casting at a chill rate of at least 36° F. per second.

12. In the method according to claim 10 wherein said operations include rolling at temperatures between 550° F. and 800° F.

13. In a method of superplastic forming wherein aluminum alloy stock is brought to superplastic forming temperature and superplastically formed into a shaped

form at superplastic forming temperature, the improvement comprising:

- (a) providing said aluminum alloy stock as an alloy comprising more than 50% aluminum and including 0.05 to 10% scandium and 0.5 to 15% magnesium;
- (b) casting said alloy at a chill rate of at least 36° F. per second;
- (c) hot rolling said alloy at temperatures not exceeding 800° F.; and
- (d) cold rolling said alloy to a cold reduction of at least 30% to provide said aluminum alloy stock for superplastic forming.

14. In the method according to claim 13 wherein said aluminum alloy contains 0.1 to 1% Sc and 1 to 7% Mg and wherein at least a substantial portion of the Mg is in solid solution at superplastic forming temperature and in combination with Sc reduces the flow stress of the alloy at superplastic forming temperature.

15. In the method according to claim 13 wherein said operations include rolling at temperatures between 550° F. and 800° F.

\* \* \* \* \*

25

30

35

40

45

50

55

60

65